

June 24, 1930.

W. E. WATKINS

1,766,417

PRODUCTION OF METAL FILMS

Filed Jan. 6, 1927



INVENTOR  
William E. Watkins  
BY  
T. C. Davis, M. M. Edwards  
ATTORNEYS

## UNITED STATES PATENT OFFICE

WILLIAM E. WATKINS, OF NEW YORK, N. Y., ASSIGNOR TO COPPER PLATE SHEET AND TUBE COMPANY, OF NEW YORK, N. Y., A CORPORATION OF NEW JERSEY

## PRODUCTION OF METAL FILMS

Application filed January 6, 1927. Serial No. 159,337.

This invention relates to methods of plating one metal with another and apparatus therefor; and more particularly to a process of forming a film of a plating metal on 5 the metal to be plated in which the plated metal is coated with a plating suspension of the plating metal in finely divided condition, or a reducible compound thereof, and passed through a furnace to heat the metal and the 10 plating suspension to form an adherent layer of the plating metal on the metal to be plated. In a prior Patent, No. 1,197,693, granted Sept. 12th, 1916, I have described and claimed a process of plating metal in which a metal 15 plating suspension, such as a mixture of an oxide of the plating metal and an oil, is applied to the metal to be plated and the metal heated to reduce the oxide and form a continuous film of the plating metal on the metal 20 to be plated. To insure the reduction of the oxide to metallic form, finely divided carbon, or other reducing agent, may be added to the metal plating suspension as disclosed and claimed in my prior Patent No. 1,197,694, 25 granted Sept. 12th, 1916. The plating metal in finely divided form may be substituted for the reducible compound and mixed with a suitable vehicle such as a semi-liquid or viscous hydrocarbon and applied to the metal 30 to be plated by coating the base with the plating suspension and heating as described in my prior patent, No. 1,197,695, granted Sept. 12th, 1916.

In plating metals according to the processes disclosed in my prior patents, the metal to be coated and the suspension thereon is heated to a temperature above the melting point of the plating metal. Thus, when ferrous metals are coated with copper, the metal 35 is heated to a temperature approximating the melting temperature of copper, or to a temperature of substantially 2000° F.

I have found that a superior plated product may be obtained if the metal is heated merely to the sintering temperature of the plating metal. Within their sintering temperature range, metals possess sufficient freedom of movement to enable them to coalesce. I have discovered that by heating the metal to 40 be plated with the metal plating suspension

thereon to the sintering temperature of the plating metal, it is possible to produce films of uniformly beautiful appearance and possessing a degree of continuity not possible when the film has been allowed to reach its 55 melting temperature. Thus, in coating ferrous metals, I propose to heat the metal with the coating applied thereto to a temperature of about 1800° F. which is sufficient to permit the copper to coalesce and form a continuous coating. I have further found that the best results are obtained if the film of plating metal is kept below its sintering temperature until the metal base has reached the proper temperature. I accordingly preheat 60 the base on which the coating film has been applied to a temperature just below the sintering temperature of the plating metal and then raise the temperature to the sintering temperature of the plating metal to form the 65 adherent film or layer on the base.

A further object of the invention is to provide a furnace having a preheating zone in which the metal base may be properly preheated before the plating film reaches its 70 sintering temperature. I accordingly provide a furnace having a preheating zone, a heat treating zone, a cooling chamber and a combustion chamber and regulate the passage 75 of the products of combustion through the furnace in such manner that the metal on which the coating has been applied is first preheated, then raised to the sintering temperature of the plating metal and then cooled before reaching the air to such a temperature 80 that it will not readily oxidize when exposed to air.

In the following illustration of the invention I have described the application of copper plating to ferrous strips. The invention 85 may be applied to the coating or plating of other metals and other plating metals may also be employed. It will be apparent that the process is equally applicable to the coating 90 of plates or sheets as well as strips.

In the accompanying drawings I have diagrammatically illustrated a type of furnace particularly useful in practicing the process and forming a part of the invention. In 100

this showing, Fig. 1 is a vertical, longitudinal, sectional view of the furnace;

Fig. 2 is a vertical, transverse, sectional view, substantially on line 2—2 of Fig. 1; 5 and,

Fig. 3 is a similar view on line 3—3 of Fig. 1.

The furnace is preferably rectangular and consists of outer walls, 1, a floor, 2, and a roof, 3, preferably lined with silocel or similar material. Within the furnace I provide side walls, 4, a floor, 5, and an inner roof, 6, of fire brick. The interior of the furnace is in 10 the form of a large rectangular chamber which is divided at the front by a separating wall, 7, of fire brick forming a preheating chamber, 8, at the top and a combustion chamber, 9, at the bottom. A burner block, 10, is arranged intermediate the ends of the 15 combustion chamber and an oil burner, 11, projects through an opening in this block. The oil burner may be supplied with the proper mixture of air and fuel in any suitable manner. The portion of the furnace in 20 the rear of the preheating zone and combustion chamber forms a heat treating zone, 12. A foot arch, 13, is arranged at the back of the partition, 7, and curves downwardly to 25 the floor of the furnace so that the products of combustion from the combustion chamber, 9, are forced to travel around this arch in entering the heat treating zone. The hot gases issuing from the combustion chamber are thus 30 divided equally by the foot arch. At the rear 35 of the furnace, I provide an opening, and a cooling chamber, 14, is connected to the furnace at this opening. The cooling chamber is of such length that the strips in passing 40 through it will be cooled to such temperature that they may then be passed into the open air without danger of oxidation. Suitable 45 rollers, 15, may be arranged at the end of the cooling chamber. A ramp, 16, may be built in the back of the furnace to prevent the gases 50 from pocketing therein. Suitable means are provided for controlling the temperature in 55 the various portions of the furnace. A stack, 17, is arranged adjacent the rear of the furnace and communicates with the interior 60 through an opening, 18. The size of this opening may be adjusted by means of slideable dampers, 19. A similar stack, 20, is arranged 65 at the rear of the cooling chamber and the flow of gases through this stack is controlled by a damper, 21. A stack, 22, is arranged adjacent 70 the front of the furnace and provided with a damper, 23. A baffle, 24, may be arranged depending from the roof of the furnace and separating the preheating zone 75 from the heat treating zone. The strip of metal to be treated is passed through the furnace in catenary form as indicated at A and as described and claimed in my copending application, Serial No. 144,685, filed October 28th, 1926. The strip is supported by the

rollers, 15, in the cooling chamber and by a suitable guide, 25, arranged at the front of the furnace.

In practicing the process the strip is first coated on one or both sides with a suspension 70 of a reducible compound of the plating metal or the metal in finely divided form and a liquid spreading medium of a reducing character which serves to protect both the plating metal and the metal to be plated during the 75 plating operation. An asphaltic base hydrocarbon oil having a viscosity of 116 has been found satisfactory as possessing the proper spreading and binding qualities while its base contains sufficient carbon to reduce 80 any oxides that may be present. When 5 grammes or less of the plating metal is to be applied to each square foot of surface, the finely divided metal and oil are mixed in the proportion of 40 per cent finely divided metal 85 and 60 per cent oil. For films of greater thickness a mixture richer in finely divided metal has been found satisfactory. The metal strip is passed through the furnace and the products of combustion from the burner, 90 11, pass from the combustion chamber around the foot arch, 13, into the heat treating chamber, 12. The temperature to be maintained in the heat treating chamber will depend upon the speed of travel of the metal being treated. 95 In a furnace of this type, approximately 25 feet long, the heat treating zone may be maintained at a temperature of 2250° F. to treat a strip 12" x .05 when the strip is traveling at a speed of 80 feet per minute. Under these 100 conditions the strip will be heated to a temperature of substantially 1800° F., in passing through the heat treating zone. A pyrometer, 26, may be placed in the heat treating zone by passing it through the wall or roof 105 of the furnace. The preheating zone may also be provided with a pyrometer, 27, and the temperature in the preheating zone should be maintained under that of the heat treating zone to prevent the plating metal from reaching 110 its sintering temperature before the metal base is at the right temperature to receive it. The furnace gases should be slightly reducing and maintained at a pressure sufficient to prevent leakage of atmospheric air in the furnace. The pressure within the furnace causes the gases to travel in both directions when they enter the heat treating zone thereby causing a portion of the gases to pass 115 through the preheating zone to the stack, 22. The baffle, 24, retards the flow of gases into the preheating zone and thus assists in maintaining a lower temperature in this zone than in the heat treating zone. The temperature of the preheating zone may also be regulated by the damper, 23. The main control of the flow of gases toward the preheating zone and the cooling chamber, 14, is accomplished by means of the sliding blocks or dampers, 19, over the opening, 18, and by properly regu- 120 130

lating the size of the opening, 18, the temperature in the various zones may be positively controlled.

The furnace may be operated at constant temperatures in the several zones and the speed of travel of the metal through the furnace may be regulated to suit the gauge of the metal being treated. The process can, of course, be modified to treat different metals and in each instance, the temperature of the heat treating zone and the speed of travel of the strip is regulated to heat the metal to the sintering temperature of the plating metal. To produce a bronze plating, the plating suspension is formed of a mixture of cupric oxide and tin oxide (or, preferably, finely divided copper, and tin oxide) in definite proportions to produce the desired bronze, to which the proper quantity of the spreading vehicle or oil is added.

The furnace construction disclosed herein forms the subject matter of a divisional application filed June 25, 1927, Serial Number 201,317.

25 I claim:

1. The herein described process consisting essentially of coating the metal to be plated with a plating suspension of the plating metal, and then heating it to the sintering 30 temperature of the plating metal for sufficient time to form an adherent film of the plating metal on the plated metal.

2. The herein described process consisting essentially of coating ferrous metal with a plating suspension of copper, and then heating it to the sintering temperature of copper for sufficient time to form an adherent film of copper on the ferrous metal.

3. The herein described process consisting 40 essentially of coating ferrous metal with a mixture of finely divided copper and an oil, and then heating it to approximately the sintering temperature of copper for a sufficient length of time to form an adherent film of copper on the ferrous metal.

4. The herein described process consisting essentially of coating the metal to be plated with a plating suspension of the plating metal, preheating it to a temperature below 50 the sintering temperature of the plating metal, and then heating it substantially to the sintering temperature of the plating metal for sufficient time to form an adherent film of the plating metal on the plated metal.

5. The herein described process consisting 55 essentially of coating the metal to be plated with a plating suspension of the plating metal in finely divided form and an oil, preheating it to a temperature below the sintering 60 temperature of the plating metal, and then heating it to substantially the sintering temperature of the plating metal to form an adherent film of the plating metal on the plated metal.

6. The herein described process consisting

essentially of coating ferrous metal with a mixture of finely divided copper and an oil, then preheating it to a temperature below the sintering temperature of copper and then heating it to substantially the sintering 70 temperature of copper for a sufficient length of time to form an adherent film of copper on the ferrous metal.

7. The herein described process consisting essentially of coating the metal to be 75 plated with a plating suspension of the plating metal and then heating the metal and the suspension to a degree just under its melting temperature for a sufficient time to form an adherent film of the plating metal on the 80 metal to be plated.

In testimony whereof I affix my signature.

WILLIAM E. WATKINS.

85

90

95

100

105

110

115

120

125

130